

## UNITED STATES PATENT OFFICE

2,090,396

FIXING COMPOSITION AND METHOD OF  
AFTERTREATING DYED MATERIALSEdward S. Chapin and Walter C. Durfee,  
Boston, Mass.No Drawing. Application December 15, 1936,  
Serial No. 115,982

23 Claims. (Cl. 8—5)

This invention relates to a fixing composition for use in, and also to a method of, aftertreating dyed materials, and especially dyed union materials, to fix the colors.

5 The invention has for an object to provide a novel fixing composition which in solution is capable of use with advantage to aftertreat dyed materials, and especially dyed union materials, and to produce resultant materials in which the  
10 colors are fast to water, to wet hot pressing against white fabrics, sometimes to perspiration, and to other conditions involving the action of water, steam, and saline solutions.

A further object of the invention is to provide  
15 a novel and improved process of treating dyed materials, and especially dyed union materials, in order to fix the colors thereof to render them fast to water, to wet hot pressing against white fabrics, sometimes to perspiration, and to other  
20 agencies which involve resistance to the action of water, steam, and saline solutions.

A further object of the invention is to provide a novel and improved fixing composition and a method of aftertreating dyed materials, and especially dyed union materials, whereby in the  
25 fixing of the colors of the dyed materials, tendering of the fibers of the material is prevented.

A further object of the invention is to provide a novel and improved fixing composition and a method of aftertreating dyed materials, and especially dyed union materials, whereby in the fixing of the colors of the dyed materials, the  
30 alteration of the shade is reduced to a minimum.

A further object of the invention is to provide a novel and improved fixing composition and a method of aftertreating dyed materials, and especially dyed union materials, whereby the colors of the dyed materials can be fixed at  
35 ordinary supply water temperature.

40 With these objects in view and such others as may hereinafter appear, the invention consists in the fixing composition and compositions hereinafter described together with the process of treating dyed materials, and especially dyed union materials, hereinafter described, and as particularly defined in the claims at the end of this specification.

45 The permanency of color in dyed fibers as to resistance to water, to wet hot pressing against white, to crocking, to perspiration, and to other

similar conditions which involve resistance to steam and saline solutions, is of great importance to the textile industries.

Especially is this true of materials and/or fabrics having mixed fibers, such as goods made from a combination of cotton and wool and similar materials and/or fabrics which may also contain rayon, silk, and other fibers. With these union materials and/or fabrics the securing of water fast results has prior to our invention required long and complicated processes, frequently resulting in off shade colors and the production of seconds. Aftertreatments have sometimes been utilized but these change the shade of the dyeings or otherwise injure the goods, and have not, in general, made the materials and/or fabrics satisfactorily water fast.

Satisfactory water fastness can be secured by the use of expensive dyes and special manufacturing and special dyeing operations. This, however, would make the fabrics too expensive for ready sale to the general trade and particularly to the medium and lower priced trade and accordingly the practise has been to use low priced, though unfast, union dyes. These union dyes are essentially mixtures of substantive (direct) dyes for coloring the cotton and the wool, as well as other fibers receptive to such dyes, and neutral dyeing (acid) dyes for coloring and toning the wool, as well as other fibers receptive to such dyes.

The method of dyeing union materials as ordinarily practised consists in running the materials and/or fabrics in a dye solution in the presence of common salt, and also adjusting the temperature of the dye-bath during the operation. The cotton and similarly acting fibers of the fabric take the direct dye in the main below the boiling point, and the wool and similarly acting fibers require more nearly a boiling for dyeing. The final step in such a process is to wash the goods in an attempt to remove the excess and unused dye. However, the results obtained are dyed products that are not fast to steeping in water, to wet hot pressing against white, to perspiration tests, and to other conditions.

Thus, the great majority of commercial fabrics of mixed fibers containing cotton, as men's wear suitings, meltons, satinets, ladies' dress goods, ladies' cloakings, ski-clothes, linings, etc., have not been dyed by the so-called union dyes prior

- to our invention in such a manner as to make them fast to water, to wet hot pressing, to perspiration, and to other conditions. As a result, where such dyed products were made up into garments, the wearers experienced staining of underneath garments and even of the body when the dyed garments became wet; and serious difficulties resulted in repressing the wet garments from the looseness of the color.
- 10 The present invention contemplates a novel fixing composition which is particularly useful in practising a process for fixing the dye or color in dyed materials, and especially dyed union materials, and which involves the aftertreatment 15 of dyed materials, and especially dyed union materials, in order to fix the dye and render it fast to water, to wet hot pressing against white fabrics, sometimes to perspiration, sometimes to wet and dry crocking, and to other conditions involving resistance to the action of water, steam, 20 and saline solutions.

The aftertreatment of dyed materials, composed of one individual fiber or of a mixture of fibers, is not new. Various water soluble metallic salts, as copper sulphate, bichromate of potash or soda, alum, and the like, alone or in conjunction with assisting chemicals, as acetic acid, bitartrate of potash, formaldehyde and the like, have been employed from time to time with the 25 object of improving the fastness of dyed materials variously to washing, to fulling, and to light. Usually the treatment has been at a boil, or at an elevated temperature, and the treatments have generally resulted in considerable changes in 30 shade of the dyeings; and also, in the case of mixed fabrics containing vegetable fiber, frequently in deterioration of the fabric. Accordingly aftertreatments of dyed materials had been practically abandoned by the art prior to our 35 invention except for the use of bichrome to after-treat or top-chrome dyed materials to improve fastness to washing, fulling, and light.

The specific requirement of fastness to water and to wet hot pressing against white fabrics, especially for dyed union goods, is of comparatively recent origin in the art and the trade. Our invention, as above set forth, comprises a novel fixing composition and a novel method of after-treatment, which is specially designed to fix the 40 dye or color in dyed materials, and especially dyed union materials, to water and to wet hot pressing against white fabrics; and it has been found at times also to fix the dye or color to perspiration, to wet and dry crocking, and to 45 other conditions involving resistance to the action of water, steam, and saline solutions.

The present fixing composition enables the aftertreatment to be carried out at relatively low temperatures, reducing the change of shade to a 50 minimum, enabling economies in both time and steam to be secured and in addition preventing the deterioration of the materials and/or fabrics.

In practising the invention, the dyed materials, and especially the dyed union materials, after 55 they have been washed clean of excess dye liquor are subjected to treatment with a preferred fixing composition.

The water soluble metallic salts, hitherto used in aftertreatment at elevated temperatures as 60 above set forth, when applied at relatively low temperatures fix the dye of dyed materials to water and to wet hot pressing against white fabrics in varying degrees. Thus bichrome fixes rather unsatisfactorily whereas alum fixes 65 sufficiently. The tendency to cause change or throw-

ing of shade is reduced by aftertreating at lower temperatures. However, the danger of tendering the fiber with those metallic salts which have a tendency to tender is not appreciably modified.

The danger of tendering the fiber, and especially the vegetable fiber in mixed fabrics, is illustrated by the effect of alum in aftertreatment. The impregnation of the fiber with alum and the subsequent liberation and concentration of the sulphuric acid, or the acid constituents of the 10 alum, during and after the drying of the goods makes tendering of the goods inevitable; and as a result the use of alum in the aftertreatment of dyed union fabrics has been generally abandoned.

The fixing composition which we prefer to employ comprises a mixture of a water soluble salt, together with one or more reagents capable of modifying the action of the water soluble salt upon the fabric so that the resulting goods are free from the deleterious effects which the water 15 soluble salts by themselves may exert in tendering the fabric, in causing color changes, in finishing the fabric, etc.

We have discovered that the desirable effects of water soluble salts in fixing the color of the 20 dye in dyed materials, and especially dyed union materials, may be successfully utilized by modifying the water soluble salt: firstly, with a reagent or reagents capable of suitably abating the acidity of the solution of the water soluble salt; secondly, 25 with a reagent or reagents capable of minimizing the change of shade; and thirdly, with other assisting reagents. We have termed these three 30 classes of reagents respectively acid-binders, shade-balancers, and assistants. The preferred 35 fixing composition contains in addition to the water soluble salts as its essential ingredient one or more representatives of all three classes of modifiers.

The number of water soluble salts and chemicals that alone or in combination will fix colors more or less, irrespective of other effects, is theoretically very great. However, practical and scientific considerations restrict the number that may be preferably employed. The water soluble 40 salts of nearly all cations, especially the metallic cations, fix colors more or less and in varying degrees. Acids, also, fix colors in varying degrees. The fixing action appears to be a metallic and/or 45 acid effect.

The fixing power of water soluble salts varies with the particular cation; and also in general increases with valence. As a rule the salts of monovalent cations have a slight fixing power; the salts of bivalent cations fix more readily; 50 and the more potent fixing salts are those of the trivalent and of the polyvalent cations.

The fixing power of acids varies with the dissociation, the more strongly dissociated acids 55 having the most effect in fixing.

Anions influence the fixing variously, but their function appears to be more an indirect one,—viz. to modify the action of the water soluble salts and chemicals. In general, the various anions influence the fixing in accordance with the principles of electrolytic dissociation and interaction. Thus salts of strong bases having acetic anions act as acid binders of salts of strong acids. The anion hydroxyl, the electrolytic opposite of the cation hydrogen, in excessive concentration is inimical to fixing.

Following is a list of salts, classified according to cations and anions, numerous representatives of which we have investigated and found to effect 75

or influence variously the fixing of the dyes of dyed materials.

A. Cations.

1. Monovalent cations.

Silver, sodium, and potassium salts, and hydrogen salts, or acids. Inasmuch as acids fix in varying degrees, the cation hydrogen is included in the list.

2. Bivalent cations.

Copper, lead, cadmium, mercury, bismuth, tin, (stannous), iron (ferrous), zinc, nickel, cobalt, calcium, barium, and magnesium salts.

3. Trivalent cations.

Aluminum, chromium, iron (ferric) salts.

4. Polyvalent cations.

Tin (stannic), titanium (tetravalent), cerium salts.

B. Anions.

Sulphates, basic sulphates, chlorides, nitrates, fluorides, acetates, formates, tartrates, citrates, tungstates, chromates, dichromates, carbonates, borates, hydroxides.

Water insoluble salts have little effect in fixing, or at the most serve to modify the fixing. Thus, whereas the water soluble chloride of barium readily fixes colors, the insoluble sulphate of barium has little if any effect. We prefer to utilize for the fixing compositions the water soluble salts.

The effect other than fixing of the various salts as above classified on dyed materials varies with the cation, the anion, the dyes, and the material. The change or throwing of the shade by after-treatment, the tendency to produce tendering of the fibers, and the liability of causing other undesirable effects varies greatly.

Practical and scientific considerations limit the number of water soluble salts that may be desirably employed as ingredients of the fixing composition: thus, high cost, as with silver, bismuth, cadmium, and cobalt salts; toxic considerations, as with lead salts; extreme tendency to tender fibers and to throw the shade, as with stannic chloride; and tendency to reduce and destroy dyes, as with stannous chloride.

The most potent fixing agents are the salts of trivalent and of polyvalent cations. After numerous experiments we have concluded that the salts of the trivalent afford the best basis for a fixing composition, that of the salts of trivalent cations the salts of aluminum are to be preferred, and in particular alum or aluminum sulphate.

The fixing composition which we prefer to employ comprises a mixture of alum or aluminum sulphate modified with suitable proportions of acid-binders, and/or shade balancers, and/or assistants.

The acid binding of the alum follows strictly the principles of electrolytic dissociation and interaction. Among acid binders may be mentioned specifically alkalies and alkaline salts, as soda ash, borax, and the like. In excess, however, these alkaline reagents tend to destroy the fixing composition. More satisfactory as acid binders are the salts of strong bases and mild organic acids, as sodium acetate, calcium acetate, sodium formate, and the like. We have found the acetates especially valuable as acid binders, and in particular calcium acetate.

The principles of shade balancing as practised in making the preferred fixing compositions is of especial importance. The dyeings of certain dyes are affected variously by different cations,—

brightened, saddened, or otherwise changed in shade. Where the dyeing of a dye is brightened on aftertreatment by certain fixing salts, as many by aluminum sulphate, and at the same time is saddened by other fixing salts, as many by chromium salts, a blending of fixing salts with opposing effects will result in a balancing of effects and consequently in a minimizing of the shade change, so that a practical process from this point of view results.

The principles of acid-binding and of shade-balancing are intimately intwined. The dyeings of many dyes are sensitive to acids and their shades are more or less changed or thrown by acid baths. Acid-binding will frequently counteract most of the change of shade caused by fixing salts that give in solution an acid bath.

In the listing above given most of the salts that fix can be utilized as shade balancers. However, in preparing the fixing compositions it is preferable to select salts where the shade differences are not too violent and consequently difficult to balance.

Many of the salts in the list above given combine all features: fixing, acid-binding, and shade-balancing. Such salts are to be preferred as modifiers of the alum. Among such salts, that we have found of especial value, are basic sulphate of chromium and calcium acetate.

Assistants that may be preferably included in the fixing composition facilitate additional desirable tendencies in the process of fixing, as evenness and penetration; and also help in producing practically required properties in the fixed result, as freedom from crock, etc. The salts of tartaric, citric acid and the like, that might be expected from general experience to promote evenness, penetration, and freedom from crock, appear to be inimical to our main purpose of fixing the colors, when used in relatively large proportions. Accordingly we have limited such additions to relatively small proportions. We prefer to use for this purpose bitartrate of potash, and in particular a high grade of argol.

Another assistant, the inclusion of which in the fixing composition is more or less optional, is common salt. This assistant appears to prevent diffusion of the dye from the fiber back into the solution, assists perhaps somewhat in the leveling and penetration of the fixing and in imparting to finished goods a desirable feel. The proportion of common salt that we prefer to use is several times the amount of the fixing reagent, and is best added in practising the process as will presently be explained.

The ease of fixing colors varies greatly with the dyes. Thus, the dyeings of the Direct Brown, Color Index No. 420, are quite readily fixed, whereas the dyeings of the Direct Blue, Color Index No. 401, which is a favorite component of cheap navy blue union mixtures, are fixed with difficulty. Ease of fixing also varies with the character of the material: dyed materials of all wool or practically all wool fix with less difficulty than dyed materials containing cotton and/or rayon, or composed entirely of cotton or rayon. The material appears to play a part, though an obscure one, in the fixing.

While the preferring fixing compositions, containing as an essential ingredient the potent fixing salt alum, are required to fix the dyeings that are hard to fix, dyeings that readily fix may be fixed by the use of a less efficient fixing composition than the preferred type by using

as an essential ingredient a less potent fixing reagent than aluminum sulphate, and indeed various salts as above classified, and modifying them in accordance with the principles as above set forth. However, it is preferable to utilize in fixing dyeings easy to fix less of the preferred fixing composition, which has specially been worked out for all-around use, for all dyes and materials.

10 Dyeings vary in their sensitiveness to acids and metals. Thus, the dyeings of the Direct Blue, Color Index No. 401, are extremely fast toward strong acids, as sulphuric and hydrochloric, and even in strongly acid baths their shades are little affected. On the other hand the dyeings of Direct Scarlet, Color Index No. 448, are sensitive toward and their shades are altered by acids, even mild organic acids.

15 In preparing the preferred fixing composition we have taken into account the various factors as above set forth. After numerous experiments we have concluded that the best all-around fixing composition for general use comprises a water soluble sulphate of aluminum, modified with suitable proportions of a basic sulphate of chromium, of calcium acetate, of argol, and of common salt.

20 The following formulas are illustrative examples of fixing compositions that may be utilized to practise the fixing of colors.

#### Formula 1

|                   | Parts |
|-------------------|-------|
| Aluminum sulphate | 60    |
| Calcium acetate   | 40    |

#### Formula 2

|                   | Parts |
|-------------------|-------|
| Aluminum sulphate | 48    |
| Calcium acetate   | 42    |
| Common salt       | 10    |

#### Formula 3

|                         | Parts |
|-------------------------|-------|
| Aluminum sulphate       | 70    |
| Basic chromium sulphate | 10    |
| Common salt             | 20    |

#### Formula 4

|                         | Parts |
|-------------------------|-------|
| Aluminum sulphate       | 48    |
| Calcium acetate         | 12    |
| Basic chromium sulphate | 12    |
| Common salt             | 28    |

#### Formula 5

|                         | Parts |
|-------------------------|-------|
| Aluminum sulphate       | 48    |
| Calcium acetate         | 12    |
| Basic chromium sulphate | 12    |
| Argols                  | 4     |
| Common salt             | 24    |

#### Formula 6

|                         | Parts |
|-------------------------|-------|
| Aluminum sulphate       | 48    |
| Calcium acetate         | 18    |
| Basic chromium sulphate | 12    |
| Argols                  | 4     |
| Common salt             | 18    |

#### Formula 7

|                         | Parts |
|-------------------------|-------|
| Aluminum sulphate       | 49    |
| Calcium acetate         | 38    |
| Basic chromium sulphate | 9     |
| Argols                  | 4     |

#### Formula 8

|                   | Parts |
|-------------------|-------|
| Aluminum sulphate | 48    |
| Soda ash          | 6     |
| Common salt       | 46    |
|                   | 5     |

#### Formula 9

|                   | Parts |
|-------------------|-------|
| Aluminum sulphate | 48    |
| Calcium acetate   | 28    |
| Tartaric acid     | 3     |
| Common salt       | 21    |

#### Formula 10

|                   | Parts |
|-------------------|-------|
| Aluminum sulphate | 48    |
| Calcium acetate   | 28    |
| Citric acid       | 2.5   |
| Common salt       | 21.5  |

While the foregoing represent typical compositions that may be employed in practise, it is pointed out that other proportions than those above given may be found advantageous.

It is evident that in accordance with the principles above set forth fixing compositions can be utilized composed essentially of other water soluble salts, as other aluminum salts and other salts as above classified, to the extent that they are similar to and analogous in action in fixing to aluminum sulphate; that other acid binders analogous to and similar in action to calcium acetate, as sodium acetate, can be employed; that other salts than basic sulphate of chromium and calcium acetate, as ferrous sulphate, similar in action and analogous in effect as shade balancers can be utilized; that other tartrates or equivalents, as Rochelle salt, similar to or analogous in action to argol can be used; and that other equivalents of common salt, as Glauber's salt, can be utilized.

It will also be understood that other water soluble salts of cations and anions not included in the above classification can be utilized as components of a fixing composition to the extent that they are similar to and analogous in action to the water soluble salts as above classified.

It will be readily understood that while each of the ingredients of the fixing composition performs a specific function as above described, there are probably actions and interactions when all are blended together and dissolved that produce practical results that are superior to those which might be ascribed separately to the individual constituents of the fixing composition. For this reason the proper proportions of the ingredients and their proper blending to produce a fixing composition contribute to most efficient use and to best results.

The preferred method of practising the use of the fixing composition will now be described, but it will be manifest to those skilled in the art that various practical variations of this method may be employed.

This process is simple to carry out and is especially distinguished by the fact that it is practised at low and convenient temperatures.

Preferably the fixing composition should be dissolved in a separate container, and in practise the fixing composition selected may be dumped into a good sized barrel and covered with several pails of cold water; the whole is well stirred up and brought to a boil and boiled for fifteen minutes, stirring occasionally. This insures the solution of the ingredients of the fixing composition and the completion of essential chemical

interactions. The barrel is then filled up with cold water and is then ready for the fixing operation.

It will be evident to those skilled in the art that this solution of the fixing composition can be made either by dissolving a previously blended fixing composition, prepared according to the above principles, or by dissolving the separate ingredients in the correct proportions. It is understood that both methods of practising the use of the fixing compositions are included in this invention. We believe it to be preferable to blend the ingredients before dissolving.

As will be developed later, acetic or formic acid can frequently be used to advantage in conjunction with the fixing composition. In such cases the acetic or formic acid, diluted in a pail of cold water, is added to the solution of the fixing composition, and the barrel is then well stirred and allowed to stand for a further five or ten minutes before using the fixing composition.

The dyed union goods having been thoroughly washed and the fixing composition having been prepared as described, the preferred process of application continues as follows. The dyeing kettle with the well washed goods is filled with cold water; ten to fifteen percent of common salt, reckoned on the weight of the goods, is added to the bath; and the goods run in this solution for five to ten minutes. This addition of salt tends to prevent the thinning of the color on the cotton and to clear up the excess dye liquor that may be left in the kettle after the washing. It is also added for reasons previously explained.

Salt may be omitted if desired in the fixing. However, we consider its use in conjoint action with the fixing composition preferable.

The fixing composition is then fed slowly to the dye-kettle in the course of ten minutes. This is to ensure uniformity of fixation and penetration of the fabric by the fixing chemicals as otherwise the action of the fixing composition in concentrated solution would be too rapid. With the gradual addition of the fixing composition, the liquor in the kettle begins to clear up from the final traces of dye, and the bath becomes virtually water white.

After the fixing composition has been fed gradually to the kettle, steam is turned on, and the bath is brought to 70° F.,—about the temperature of ordinary supply water in summer; and the fixing then continued for fifteen to twenty minutes. Running at a higher temperature, as 100–110° F., may be advisable with certain fabrics difficult to penetrate. The conditions of temperature best suited to any particular fabric can be determined by practical trials.

The quantity of fixing composition required to make dyed union fabrics fast to water, wet hot pressing against white fabrics, sometimes to perspiration, and to other conditions involving the action of water, steam, and saline conditions, depends on the depth of the dyeing and the character of the dyes. Light dyeings will require less of the fixing composition than medium and heavy shade dyeings, and as has already been pointed out certain dyes fix relatively readily and others are hard to fix. Depending on the varying circumstances of the dyeing, the amounts of fixing composition will vary from 1½ to 6 pounds per one hundred pounds of dyed goods to be fixed.

In fixing it is advisable to use more fixing composition than will exactly fix the dye of the dyed goods. Accordingly, after fixing as above described, there will be an excess of fixing composi-

tion in the liquor of the kettle and also certain amounts of fixing composition liquor loosely held in and on through the fibers of the fabric. It is essential to wash out of the bath and fabric the excess of fixing composition. There are several reasons for this, including a slight further elimination of acidity to fully insure safety in drying, and more particularly for the reason to be presently explained. In this regard we found in some examples, which appeared to be satisfactory, that the proper degree of washing was attained when the acidity of the materials and/or fabrics had been decreased to a point on the pH scale in the vicinity of 5 to 6. This frequently requires as thorough a washing as is commonly given after 15 dyeing.

The reasons for these precautions become very manifest in the fixing of heavy weight fabrics and especially those that after drying and shearing have to be heavily pressed. With such goods there is always a tendency to stick to the presses, causing wrinkles, streaks or even eventually tearing of the fabric. This tendency is accentuated if an excess of fixing composition is left in the goods, as can occur if they are not sufficiently washed after fixing.

The principles enunciated for heavy weight fabrics apply, though in a lesser degree, to lighter weight goods. The amount and degree of precautions necessary for any fabric can be determined by practical trials.

Acetic acid or formic may be used in the fixing process for various reasons. First, to neutralize any alkali that may be present in the dyed goods. Alkali in the goods may come variously from insufficient washing after fulling, or from the dye, or from alkali used with the salt in dyeing. The presence of alkali in the goods to be fixed tends to destroy the balances of the fixing composition. When alkali is detected in the goods it should be neutralized, and the acetic or formic acid is preferably added with the salt prior to the adding of the fixing composition to the bath. Another reason for the use of acetic or formic acid is to reduce to a minimum the cost of fixing. It has been found that the addition of acetic or formic acid to the solution of the fixing composition makes it possible with some materials, as heavy meltons, to reduce the amount of fixing composition required to fasten the dyeing to water and to other conditions above indicated. Acetic or formic acid, furthermore, assists in reducing the "sticking" tendencies of goods in pressing.

In the above description of the practising of the use of the fixing compositions, it was recommended to use an excess of fixing composition and to wash thoroughly after fixing. Experience has shown that in general the amount of fixing composition can be appreciably reduced and the time required for washing eliminated by the use of specially prepared fixing compositions. Such a fixing composition is illustrated by Formula #7 as above set forth. These special fixing compositions are prepared with relatively larger proportions of acid binding ingredients, so that the acid of the alum, or other metallic salt, will be completely buffered even when not washed from the goods, the same principles being involved as in the preparation of all the fixing compositions as above set forth.

While a distinctive feature of the practising of the use of the fixing compositions is their application at low temperatures, they may be also utilized at elevated temperatures, even at a boil, with certain materials to advantage.

It will be understood that the words "cotton" and "wool", as used throughout the specifications and claims are typical of and intended to define fibers that act in a general way similarly to "cotton" and "wool"; and that the words "cotton and wool, union materials and/or fabrics" are representative of and intended to define a great variety of commercial union materials and/or fabrics, consisting of two or more different fibers, and 10 composed in a general way similarly to "cotton and wool union materials and/or fabrics". Thus, rayon behaves in a general way similarly to cotton; and mohair to wool; and union materials and/or fabrics composed of cotton, rayon, and 15 wool; cotton and mohair; cotton, wool, and silk; and various other blends may be fixed most efficiently by the fixing compositions above described.

In this application the word materials is intended to mean in addition to union materials, single materials such as wool, cotton, rayon, silk, and leather, which may be dyed unfast to one or more of the above requirements, and which can be fixed advantageously by the use of our fixing 25 compositions.

The described use of the preferred types of fixing compositions possesses a number of important commercial advantages as will be appreciated from the above description. These may 30 be summed up as producing dyed products, and especially dyed union products, the dyeings of which are fast to water, to wet hot pressing against white, sometimes to perspiration, and to other similar agencies. In addition they prevent the 35 tendering of the cotton and reduce change of shade to a minimum. A further practical advantage is that the specks of dyed union materials and/or fabrics are not stripped in the use of our preferred types of fixing compositions, as in the 40 case of other fixing agents. The process can be carried out in a comparatively short period of time, and at comparatively low temperatures, thus effecting economies in time and steam as compared with previous processes; and also safeguarding 45 the texture of goods which are more or less damaged by long treatments, particularly at elevated temperatures, and therefore could not, prior to our invention, be safely and satisfactorily fixed.

Another important practical advantage resulting from the use of the preferred fixing compositions, as above set forth, is comparative immunity from undesirable accidental effects in the dye-house. The preferred fixing compositions and especially those for leaving in the goods, and the 50 method of practising their use, as above set forth, appear to be virtually "fool-proof". Thus, if in their practising the temperature accidentally goes high, or if too much of the fixing composition is weighed out, or other and similar occasional 55 errors or infractions of the preferred method should occur, results in the main will be satisfactory.

As used throughout the specifications and claims, the term "fix" is intended to define the 60 rendering of the dye in the dyed fibers permanent with respect to its resistance to water, to wet hot pressing against white, sometimes to perspiration, and to other similar agencies which involve resistance to steam and saline solutions.

70 The term "modifying" as used by us in the specifications and claims is intended to define and include acid-binding shade-balancing, abating, modifying either in whole or in part, buffering, and the other described effects upon the fixing 75 agent and the goods.

This application is a continuation-in-part of our applications Serial Nos. 61,760 and 61,761 filed January 31, 1936.

While the preferred embodiment of the invention has been illustrated and described, it will be understood that the invention may be embodied in other forms within the scope of the following claims.

Having thus described the invention, what is claimed is:

1. A fixing composition for use in the after-treatment of dyed materials, including dyed union materials, comprising a fixing reagent having as an essential component a water soluble metallic salt, which has a tendency to tender vegetable fiber, and an acid binding agent. 10

2. A fixing composition for use in the after-treatment of dyed materials, including dyed union materials, comprising a fixing reagent having as an essential component a water soluble sulphate 15 of aluminum and an acid binding agent. 20

3. A fixing composition for use in the after-treatment of dyed materials, including dyed union materials, comprising a fixing reagent having as an essential component a water soluble sulphate 25 of aluminum and an acid binding agent including an acetate. 25

4. A fixing composition for use in the after-treatment of dyed materials, including dyed union materials, comprising a fixing reagent having as 30 an essential component a water soluble sulphate of aluminum and an acid binding agent including calcium acetate. 30

5. A fixing composition for use in the after-treatment of dyed materials, including dyed union materials, comprising a fixing reagent having as an essential component a water soluble metallic salt, which has a tendency to throw the shade, and a shade balancing agent comprising a water soluble metallic salt. 35

6. A fixing composition for use in the after-treatment of dyed materials, including dyed union materials, comprising a fixing reagent having as an essential component a water soluble metallic salt of a trivalent cation, which has a tendency 45 to throw the shade, and a shade balancing agent comprising a water soluble metallic salt. 45

7. A fixing composition for use in the after-treatment of dyed materials, including dyed union materials, comprising a fixing reagent having as an essential component a water soluble sulphate of aluminum and a shade balancing agent comprising a water soluble metallic salt. 50

8. A fixing composition for use in the after-treatment of dyed materials, including dyed union materials, comprising a fixing reagent having as an essential component a water soluble sulphate of aluminum and a shade balancing agent comprising a basic chromium sulphate. 55

9. A fixing composition for use in the after-treatment of dyed materials, including dyed union materials, comprising a fixing reagent having as an essential component a water soluble metallic salt, which has a tendency to tender vegetable fiber and to throw the shade, and an acid binding agent, and a shade balancing agent comprising a water soluble metallic salt. 60

10. A fixing composition for use in the after-treatment of dyed materials, including dyed union materials, comprising a fixing reagent having as an essential component a water soluble sulphate of aluminum and an acid binding agent, and a shade balancing agent comprising a water soluble metallic salt. 70

11. A fixing composition for use in the after- 75

treatment of dyed materials, including dyed union materials, comprising a fixing reagent having as an essential component a water soluble metallic salt, which has a tendency to tender 5 vegetable fiber and to throw the shade, and a combined acid binding and shade balancing agent comprising a water soluble metallic salt.

12. A fixing composition for use in the after-treatment of dyed material, including dyed union 10 materials, comprising a fixing reagent having as an essential component a water soluble sulphate of aluminum and a combined acid binding and shade balancing agent comprising a water soluble metallic salt.

15 13. A fixing composition for use in the after-treatment of dyed materials, including dyed union materials, comprising a major portion of a water soluble sulphate of aluminum and a minor portion of basic chromium sulphate.

20 14. A fixing composition for use in the after-treatment of dyed materials including dyed union materials comprising a water soluble sulphate of aluminum, calcium acetate and basic chromium sulphate.

25 15. A fixing composition for use in the after-treatment of dyed materials including dyed union materials comprising a water soluble sulphate of aluminum, calcium acetate, basic chromium sulphate and an argol.

30 16. In the method of treating washed, dyed materials, the step comprising subjecting the dyed materials, including dyed union materials, to treatment with a solution of a fixing reagent having as an essential component a water soluble metallic salt, which has a tendency to throw the shade, and a shade balancing agent comprising a water soluble metallic salt.

35 17. In the method of treating washed dyed materials the step comprising subjecting the dyed materials, including dyed union materials, to treatment with a solution of a fixing reagent having as an essential component a water soluble metallic salt, which has a tendency to tender vegetable fiber and to throw the shade, and an acid binding agent, and a shade balancing agent comprising a water soluble metallic salt.

40 18. In the method of treating washed dyed materials, the step comprising subjecting the dyed materials, including dyed union materials, to treatment at relatively low temperature with 45 a solution of a fixing reagent having as an es-

sential component a water soluble metallic salt, which has a tendency to tender vegetable fiber and to throw the shade, and an acid binding agent, and a shade balancing agent comprising a water soluble metallic salt.

5 19. In the method of treating washed dyed materials, the step comprising subjecting the dyed materials, including dyed union materials, to treatment at relatively low temperatures with a solution of a fixing reagent having as an essential component a water soluble sulphate of aluminum and an acid binding agent, and a shade balancing agent comprising a water soluble metallic salt.

10 20. In the method of treating washed dyed materials, the step comprising subjecting the dyed materials, including dyed union materials, to treatment with a solution of a fixing reagent having as essential components a water soluble sulphate of aluminum, an acid binding agent comprising a water soluble metallic salt, a shade balancing agent, and a substantial proportion of salt.

15 21. In the method of treating washed dyed materials, the step comprising subjecting the dyed materials to treatment with a solution of a fixing reagent having as an essential component a water soluble metallic salt which has a tendency to tender vegetable fiber and to throw the shade, an acid binding agent, a shade balancing agent comprising a water soluble metallic salt and a substantial proportion of common salt.

25 22. In the method of treating washed dyed materials, the step comprising subjecting the dyed materials to treatment with a solution of a fixing reagent having as an essential component a water soluble metallic salt which has a tendency to tender vegetable fiber and to throw the shade, an acid binding agent, a shade balancing agent comprising a water soluble metallic salt and a mild organic acid.

30 23. In the method of treating washed dyed materials, the step comprising subjecting the dyed materials including dyed union materials to treatment with a fixing reagent having as an essential component a water soluble sulphate of aluminum, an acid binding agent and a shade balancing agent comprising a water soluble metallic salt.

35 EDWARD S. CHAPIN. 50  
WALTER C. DURFEE.